

# United States Patent [19]

Kanehira et al.

[11] 3,914,497

[45] Oct. 21, 1975

[54] NON-WOVEN BATTS POSSESSING  
EXCELLENT TENSILE STRENGTH, TEAR  
STRENGTH AND INITIAL MODULUS

[75] Inventors: Hiroshi Kanehira, Kurashiki; Syozi  
Kuroasaki, Okayama, both of Japan

[73] Assignee: Kuraray Co., Ltd., Kurashiki, Japan

[22] Filed: Sept. 11, 1973

[21] Appl. No.: 396,136

## [30] Foreign Application Priority Data

Sept. 14, 1972 Japan..... 47-72427

[52] U.S. Cl. .... 428/288; 156/181; 156/283

[51] Int. Cl.<sup>2</sup> .... B32B 5/28; D04B 1/58

[58] Field of Search ..... 161/170, 150, 157, 252;  
156/306, 181, 283

## [56] References Cited

### UNITED STATES PATENTS

|           |         |              |         |
|-----------|---------|--------------|---------|
| 3,049,466 | 8/1962  | Erlich ..... | 161/150 |
| 3,117,056 | 1/1964  | Katz .....   | 161/170 |
| 3,276,944 | 10/1966 | Levy .....   | 161/157 |
| 3,322,607 | 5/1967  | Jurry .....  | 161/170 |

|           |        |                |         |
|-----------|--------|----------------|---------|
| 3,393,685 | 7/1968 | Mumpower ..... | 161/170 |
| 3,501,369 | 3/1970 | Derlich .....  | 161/170 |
| 3,502,538 | 3/1970 | Petersen ..... | 161/170 |
| 3,671,383 | 6/1972 | Sakata .....   | 161/252 |

## FOREIGN PATENTS OR APPLICATIONS

|           |         |       |
|-----------|---------|-------|
| 3,511,784 | 8/1960  | Japan |
| 4,226,830 | 12/1967 | Japan |

Primary Examiner—George F. Lesmes

Assistant Examiner—Ellis P. Robinson

Attorney, Agent, or Firm—Bacon & Thomas

[57]

## ABSTRACT

Non-woven batts possessing excellent tensile strength, tear strength and initial modulus are comprised of isotactic polypropylene substrate fibers bonded together by an ethylene-propylene random copolymer, said copolymers advantageously having an ethylene content of between about 3 to 20 mole percent. The ethylene-propylene random copolymer is desirably present in the proportion of approximately 5 to 75 weight percent relative to the weight of the isotactic polypropylene fibers.

4 Claims, No Drawings

**NON-WOVEN BATTES POSSESSING EXCELLENT  
TENSILE STRENGTH, TEAR STRENGTH AND  
INITIAL MODULUS**

**BACKGROUND OF THE INVENTION**

**1. Field of the Invention**

This invention relates to novel non-woven batts, e.g., non-woven fabrics, comprised of isotactic polypropylene substrate fibers which are bonded together by an ethylene-propylene random copolymer, said copolymer advantageously having an ethylene content of approximately 3 to 20 mole percent. These novel batts possess excellent tensile strength, tear strength and initial modulus. The non-woven batts of this invention exhibit particularly advantageous properties when in the configuration of a spun-bonded, non-woven batt. 15

**2. Description of the Prior Art**

Spun-bonded, non-woven batts or fabrics have been developed with superior tensile strength as compared to non-woven batts of staple fibers. See U.S. Pat. No. 3,338,992 and U.S. Pat. No. 3,341,394. However, non-woven batts irreproachable from a practical viewpoint cannot be obtained according to the methods disclosed therein regardless of the polymer selected. The prior art teaches a method of incorporating small amounts of adhesive fiber into the substrate fibers with subsequent melting of the adhesive fibers to effect bonding of the substrate fibers. For instance, it is taught that polycaproamide (Nylon 6) fibers or a copolymer or mixture of polycaproamide and polyhexamethylene adipamide (Nylon 66) can be employed as the adhesive fibers for polyhexamethylene adipamide substrate fibers, and that fibers comprising a copolymer of ethylene terephthalate and ethylene isophthalate, or polyethylene terephthalate fibers having a low degree of molecular orientation, can be utilized as the adhesive fibers for polyethylene terephthalate substrate fibers. 25

Furthermore, in U.S. Pat. No. 3,322,607 and U.S. Pat. No. 3,276,944, it is disclosed that self-bonded, non-woven fabrics may be prepared from isotactic polypropylene or copolymers composed mainly of ethylene and propylene. However, as is clear from the results shown in the comparative examples, infra, these self-bonded, non-woven batts do not possess the excellent mechanical properties which can be obtained according to this invention. 45

Still further, Japanese Patent Publication No. 11784/60 and Japanese Patent Publication No. 26830/67 disclose that the tenacity of shaped articles prepared from polypropylene fibers can be improved by forming thereon a coating of an ethylene-propylene copolymer containing an organic peroxide, a curing agent and the like. The ethylene content of the ethylene-propylene copolymer used in this proposal ranges from 20 to 80 mole percent, with 55 mole percent the norm. 50

Although various attempts have been made to improve the tenacity of non-woven fabrics composed mainly of isotactic polypropylene fibers described hereinabove, bonded non-woven batts, e.g., non-woven fabrics and the like, obtained according to these methods are still unsatisfactory as illustrated in the following comparative examples. 55

In addition to the foregoing methods incorporating adhesive fibers with substrate fibers, there have also been employed for similar purpose methods of spraying an adhesive rubber latex onto non-woven batts or im- 60

mersing non-woven batts in a rubber latex bath, as well as methods incorporating easily-soluble fibers in such non-woven batts and subsequently selectively dissolving those fibers with appropriate selective solvent. 5 However, these methods are not practical as bonding procedures are complicated and manufacturing costs are high.

**SUMMARY OF THE INVENTION**

Accordingly, it is the primary object of this invention to obviate deficiencies in the prior art thereby yielding a non-woven batt of polypropylene fibers bonded together by an ethylene-propylene random copolymer, which batt exhibits excellent mechanical properties. 10

It is another object of the present invention to provide such a non-woven batt wherein polypropylene continuous filaments are employed to yield a spun-bonded, non-woven batt. 15

It has now been found that among the bonding methods detailed hereinabove, the method of incorporating a component capable of melting (hereinafter referred to as the "hot melting component" and represented by the ethylene-propylene copolymer) along with the substrate fibers, and melting that component to bond the substrate fibers, is most desired; and that in the case of isotactic polypropylene substrate fibers, optimum results are obtained when an ethylene-propylene random copolymer, especially one having an ethylene content of approximately 3 to 30 mole percent, is employed as the adhesive component in an amount of approximately 5 to 75 weight percent relative to the weight of the substrate fibers. 20 30

**DETAILED DESCRIPTION OF THE INVENTION**

The substrate fibers of the non-woven batts of this invention are comprised of isotactic polypropylene. While the lengths of the substrate fiber is not particularly critical, e.g., fiber length, staple fiber length, etc., in order to obtain non-woven batts broadly applicable to various uses and possessing high practical utility, it is desirable that the non-woven batts comprise spun-bonded continuous filaments. 35

According to this invention, a hot melting component is incorporated in the non-woven batt in order to improve the mechanical properties thereof and it is the most prominent feature of this invention that a specific adhesive component be utilized. Furthermore, it is indispensable that this hot melting component be a random copolymer of ethylene and propylene monomers, if the intended objects of this invention are to be attained. 40 50

If an ethylene-propylene block copolymer were to be incorporated as the hot melting component, even if the ethylene content be within the range specified by this invention, substantial improvement in mechanical properties would not be realized. The physical properties of such a block copolymer resemble those of a blend of polypropylene and polyethylene and neither polymer is itself suited as the adhesive component. 55

Not only is it important to this invention that the adhesive be a random copolymer, it is also necessary that the ethylene content of the random copolymer be lower than the propylene content, i.e., be lower than 50 percent, and most preferably be within the range of from 3 to 20 mole percent. Should the ethylene content be lower than 3 mole percent, the bonding operation experiences difficulties due to the small difference be- 60

tween the melting points of the hot melting component and the substrate fibers. Should the ethylene content exceed 20 mole percent, particularly the 50 mole percent or more illustrated in Japanese Patent Publication No. 11784/60, the elastic properties of the batt reside in the hot melting component and, therefore, marked degradation of the initial modulus is observed. The hot melting component according to the invention is advantageously crystalline and has a melting point at least 10°C. lower than the melting point of the substrate fibers; the most preferred ethylene content of the hot-melting component utilized in this invention is about 4 to 6 mole percent.

While the hot melting component may take any one of a number of physical forms, for instance, fiber, film or powder, it is indispensable that the hot melting component be incorporated into the isotactic polypropylene substrate fibers in the approximate proportion of from 5 to 75 weight percent relative to the weight of the substrate fibers. When the amount of the hot melting component is less than 5 weight percent, no prominent improvement of mechanical properties, particularly tensile strength, is observed; should the amount of the hot melting component exceed 75 weight percent, the tear strength is drastically reduced. It is preferred that the hot melting component be incorporated in an amount of approximately 7 to 30 weight percent relative to the weight of the substrate fibers to yield non-woven batts of high tenacity, high tear strength and high initial modulus.

In accordance with the preferred embodiment of this invention, both the hot melting component and the substrate are in fibrous form, most preferably in filamentary form. To facilitate the accurate monitoring of the proper proportions of each component, both may be extruded from the same spinneret or, alternatively, from adjacent spinnerets. In either case, the fibers filaments or yarn thus extruded are accumulated on a receiving surface disposed therebelow. To aid in such deposition technique, there can be disposed below the spinneret head either a filament or yarn suction device or a device for generating a charge of static electricity or electrostatic field. It is also within the ambit of this invention to extrude the filaments from a large diameter orifice spinneret in combination with the utilization of high pressure fluids. Optionally, the hot melting component may be added in the form of either fibers, staple fibers or powder, or the like, to the isotactic polypropylene substrate fibers and intimately admixed therewith, most desirably such forms of the hot melting component are simply added to an existing non-woven batt comprised of the isotactic polypropylene fibers on the surface of the said batt or at the interior thereof, or both.

Further in attaining the objects of this invention, the hot melting component is melted by means of any suitable heat treatment and then the batt is subjected to pressure, desirably concurrently therewith, to effect the bonding between and among the substrate fibers and thus consolidate the batt. The heat treatment should be carried out at a temperature between not higher than the melting point of the substrate fiber and lower than that of the hot melting component by up to 20°C. or less. Preferably, this treatment is conducted at a temperature within the range of the melting point of the substrate fiber and higher than 10°C. lower than the melting point of the hot melt component. Conventional

hot pressing techniques, i.e., with hot rolls or hot presses, may be employed for this purpose. For example, there can be employed that method comprising inserting the non-woven batts incorporating the hot melting component between hot pressure plates or hot pressure rollers to melt the said hot melting component and simultaneously consolidate the fabric. By this particular hot press treatment, the ethylene-propylene random copolymer component incorporated in the non-woven batt is substantially completely melted and the substrate fibers are thence bonded to one another, concomitantly resulting in the disappearance of any "fluff" from the surface of the said non-woven batt. Consequently, there is thus obtained a non-woven batt having a high tensile strength, a high tear strength and a high initial modulus.

As will be seen from the examples and comparative examples which follow, the isotactic polypropylene non-woven batts of this invention exhibit mechanical properties much higher than those which can be attained with non-woven batts of isotactic polypropylene consolidated by means of hot melt techniques other than those specified according to the invention. Thus, in order to further illustrate the invention and the advantages thereof, such specific examples are given, it being understood that the same are intended merely as illustrative and in no wise limitative.

### EXAMPLES 1 AND 2 AND COMPARATIVE EXAMPLES 1 TO 9

Isotactic polypropylene having a melt index of 30 was extruded at a rate of 80 g/min from a spinneret maintained at 265°C. and having 20 orifices, each with a diameter of 1.2 mm. An ethylene-propylene random copolymer having an ethylene content of 5 mole percent and a melt index of 5 was extruded at a rate of 16 g/min from a spinneret maintained at 280°C. and having 4 orifices, each of the same diameter as above. These extruded filaments (yarn) were all stretched by means of corresponding, individual take-up rollers positioned 5 cm below each spinneret. The take-up rate was about 3800 m/min in the case of the polypropylene yarn and about 1800 m/min in the case of the copolymer yarn. Both types of the stretched yarns were next introduced into an air nozzle disposed below the take-up rollers and subsequently deposited on a moving metal wire net having a suction machine at the lower portion thereof. Thence was obtained a soft, flexible non-woven fabric having a weight of 100 g/m<sup>2</sup>. The non-woven fabric thus formed was hot-pressed at 158°C. for 3 minutes under a pressure of 0.5 Kg/cm<sup>2</sup> between metal wire nets of mesh, to thereby melt the ethylene-propylene random copolymer filaments present in the non-woven fabric. It was observed that uniform bonding was attained throughout the sectional direction of the batt with no surface fluffs thereon. Properties of the resultant non-woven fabrics are shown in Table 1.

In accordance with the foregoing method, non-woven fabrics were prepared by employing various hot melting polymers (in each case, the weight of the non-woven fabric was 100 g/m<sup>2</sup>). Properties of these non-woven fabrics are also shown in Table 1. In comparative Examples 4 and 7, the hot melting polymer was employed in powder form.

TABLE 1

| Ex. No.           | Hot Melting Polymer                                                 | Mixing Ratio of Hot Melting Polymer to Isotactic Polypropylene Fibers (parts) | Melting Treatment |   | Thickness of Non-Woven Fabrics after Melting Treatment (mm) | Tensile Strength (Kg/cm) | Initial Modulus (Kg/mm <sup>2</sup> ) | Tear Strength (Kg) | Remarks (bonding conditions)   |
|-------------------|---------------------------------------------------------------------|-------------------------------------------------------------------------------|-------------------|---|-------------------------------------------------------------|--------------------------|---------------------------------------|--------------------|--------------------------------|
| Ex. 1             | ethylene-propylene random copolymer (ethylene content; 5 mole %)    | 20                                                                            | 158               | 3 | 0.30                                                        | 8.0                      | 15.2                                  | 6.2                | no fluffs on the sheet surface |
| Ex. 2             | ditto (ethylene content; 16 mole %)                                 | 10                                                                            | 155               | 3 | 0.32                                                        | 7.5                      | 11.0                                  | 8.3                | ditto                          |
| Comparative Ex. 1 | ditto (ethylene content; 5 mole %)                                  | 4                                                                             | 158               | 3 | 0.38                                                        | 29                       | 13.6                                  | 7.1                | fluffs on the sheet surface    |
| Comparative Ex. 2 | ditto (ethylene content; 5 mole %)                                  | 85                                                                            | 158               | 3 | 0.28                                                        | 7.0                      | 16.1                                  | 3.0                | film-like (excessive bonding)  |
| Comparative Ex. 3 | ditto (ethylene content; 2 mole %)                                  | 10                                                                            | 158               | 3 | 0.40                                                        | 2.4                      | 13.0                                  | 7.1                | insufficient bonding           |
|                   |                                                                     |                                                                               | 165               | 3 | 0.25                                                        | 5.0                      | 17.4                                  | 2.0                | film-like, semi-transparent    |
| Comparative Ex. 4 | ditto (ethylene content; 28 mole %)                                 | 10                                                                            | 140               | 3 | 0.35                                                        | 5.2                      | 6.7                                   | 8.5                |                                |
| Comparative Ex. 5 | ethylene-propylene block copolymer (ethylene content; 7 mole %)     | 20                                                                            | 160               | 3 | 0.40                                                        | 2.5                      | 13.6                                  | 7.1                | fluffs on the sheet surface    |
| Comparative Ex. 6 | isotactic polypropylene having low molecular orientation            | 10                                                                            | 160               | 3 | 0.40                                                        | 3.6                      | 13.3                                  | 8.0                | insufficient bonding           |
| Comparative Ex. 7 | atactic polypropylene                                               | 10                                                                            | 165               | 3 | 0.25                                                        | 5.0                      | 16.5                                  | 2.5                | film-like                      |
| Comparative Ex. 8 | high density polyethylene                                           | 10                                                                            | 145               | 3 | 0.41                                                        | 4.0                      | 9.6                                   | 7.5                |                                |
| Comparative Ex. 9 | ethylene-vinyl acetate copolymer (vinyl acetate content; 30 mole %) | 10                                                                            | 140               | 3 | 0.42                                                        | 5.0                      | 7.4                                   | 6.1                |                                |

As is apparent from the results shown in Table 1, only non-woven fabrics according to this invention have excellent mechanical properties in the sense of tensile strength, tear strength and initial modulus. Differences in values relative to these properties, between the non-woven fabrics obtained in the Examples according to this invention and those obtained in the Comparative Examples, are markedly probative.

### EXAMPLES 3 AND 4

The procedures of Examples 1 and 2 were repeated in the same manner, except that the hot melting component was not incorporated in the form of filaments but was mixed in the form of staple fibers with the non-woven fabrics of isotactic polypropylene filaments (Example 3) or was sprinkled in the form of powder onto the non-woven fabrics of isotactic polypropylene filaments (Example 4). The results of these latter experiments are shown in Table 2.

TABLE 2

| Example No.                                                    | Example 3                                                        | Example 4                                                         |
|----------------------------------------------------------------|------------------------------------------------------------------|-------------------------------------------------------------------|
| Hot Melting Polymer                                            | ethylene-propylene random copolymer (ethylene content; 4 mole %) | ethylene-propylene random copolymer (ethylene content; 10 mole %) |
| Mixing Ratio of Hot Melting Polymer to Isotactic Polypropylene | 25                                                               | 15                                                                |

TABLE 2—Continued

| Example No.                                                 | Example 3                                                        | Example 4                                                         |
|-------------------------------------------------------------|------------------------------------------------------------------|-------------------------------------------------------------------|
| Hot Melting Polymer                                         | ethylene-propylene random copolymer (ethylene content; 4 mole %) | ethylene-propylene random copolymer (ethylene content; 10 mole %) |
| Fibers (parts)                                              |                                                                  |                                                                   |
| Melting Treatment Temperature (°C)                          | 160                                                              | 160                                                               |
| Melting Treatment Time (min.)                               | 3                                                                | 3                                                                 |
| Thickness of Non-Woven Fabrics after Melting Treatment (mm) | 0.29                                                             | 0.31                                                              |
| Tensile Strength (Kg/cm)                                    | 7.8                                                              | 7.4                                                               |
| Initial Modulus (Kg/mm <sup>2</sup> )                       | 15.5                                                             | 13.0                                                              |
| Tear Strength (Kg)                                          | 6.6                                                              | 6.2                                                               |

As will be seen from the results shown in Table 2, non-woven fabrics having properties equivalent to those non-woven fabrics obtained by the spun-bonding method can be obtained by other various methods according to the invention.

### COMPARATIVE EXAMPLES 10 AND 11

The procedures of Example 1 were repeated in the same manner, except that in one instance the hot melting filaments of the ethylene-propylene random copolymer having an ethylene content of 5 mole percent were not incorporated, namely, isotactic polypropylene

filaments alone were employed (Comparative Example 10), and in the second instance the hot melting filaments alone were employed, namely, the isotactic polypropylene filaments were not used (Comparative Example 11). Mechanical properties of the obtained non-woven fabrics (each being a self-bonded non-woven fabric) are shown in Table 3.

TABLE 3

| Example No.                           | Comparative Example 10 | Comparative Example 11 |
|---------------------------------------|------------------------|------------------------|
| Tensile Strength (Kg/cm)              | 3.2                    | 2.3                    |
| Initial Modulus (Kg/mm <sup>2</sup> ) | 16.8                   | 10.6                   |
| Tear Strength (Kg)                    | 5.0                    | 4.9                    |

As is seen from the results of the foregoing Examples and Comparative Examples, the non-woven fabrics specified by this invention have excellent mechanical properties superior to those exhibited by conventional non-woven fabrics. If but one of the critical features of this invention is not satisfied, the intended objects of the invention cannot be attained.

While the invention has been described and illustrated with reference to certain preferred embodiments thereof, those skilled in the art will appreciate that various modifications, changes, omissions and substitutions

can be made without departing from the spirit of the invention. It is intended, therefore, that the invention be limited only by the scope of the following claims.

What is claimed is:

- 5 1. A non-woven batt having high tensile strength, high tear strength and high initial modulus, which comprises a batt of isotactic polypropylene substrate fibers bonded together by means of an ethylene-propylene random copolymer wherein the ethylene content of said ethylene-propylene random copolymer is from 4 to 10 6 mole percent and is present in the approximate proportion of 5 to 75 weight percent relative to the weight of said isotactic polypropylene substrate fibers.
- 15 2. A non-woven batt according to claim 1, wherein said ethylene-propylene random copolymer is present in the approximate proportion of 7 to 30 weight percent relative to the weight of said isotactic polypropylene substrate fibers.
- 20 3. A non-woven batt according to claim 1, wherein said isotactic polypropylene component is in the form of continuous filaments.
- 25 4. A non-woven batt according to claim 2, wherein said isotactic polypropylene component is in the form of continuous filaments.

\* \* \* \*

30

35

40

45

50

55

60

65